

W. L. WEST.

CARBON PAPER.

APPLICATION FILED AUG. 6, 1908.

910,887.

Patented Jan. 26, 1909.



1/3

Fig. 1.



Fig. 2.

Witnesses

Gilson Shaffer  
V. E. Loveland.

<sup>Inventor</sup>  
William L. West  
By Edward R. German

Attorney

# UNITED STATES PATENT OFFICE.

WILLIAM L. WEST, OF FRANKLIN, PENNSYLVANIA.

## CARBON-PAPER.

No. 910,887.

Specification of Letters Patent.

Patented Jan. 26, 1909.

Application filed August 6, 1908. Serial No. 447,341.

*To all whom it may concern:*

Be it known that I, WILLIAM L. WEST, citizen of the United States, residing at Franklin, in the county of Venango and State of Pennsylvania, have invented certain new and useful Improvements in Carbon-Paper, of which the following is a specification, reference being had therein to the accompanying drawing.

10 My invention relates to improvements in carbon paper, the preparation of which, and the composition for coating same are herein fully set forth, and illustrated in the accompanying drawings in which Figure 1 shows a 15 plan view of the carbon paper and Fig. 2 is a section thereof.

Similar numerals refer to similar parts in both views.

My improved carbon paper is produced as follows: I first coat the paper 1 with an impression-yielding composition 2, composed of printer's copying ink 70 per cent., glycerin 10 per cent., spirits of turpentine 10 per cent., spirits of camphor 10 per cent., which may be 25 applied to the paper by any approved method. Immediately after the application of said coating, before the same has become set or dried, I apply upon said coating a thin coating 3 of finely powdered soap,—preferably white castile soap, though I do not wish to be understood as confining myself specifically to this particular kind of soap. After 30 my impression-yielding coating has been applied to the paper, it is of substantially the

same nature as the various makes of paper in common use, but after the powdered soap has been applied, it is practically non-smutting; that is, the impression-yielding coating will not rub off when the paper is handled, neither will it smut or soil the interleaved 40 copies which are being made by it, as many other brands of carbon paper will do, which is due to the fact that the powdered soap, being applied to the first coating while it is still damp, becomes to a certain extent incorporated therewith, and forms a thin saponaceous film over the same.

Having thus described my invention, what I claim and desire to secure by Letters Patent, is—

1. A carbon paper having a thin coating of finely powdered soap overlying the impression-yielding substance.
2. A carbon paper having an impression-yielding coating, and a saponaceous coating 55 overlying said impression-yielding coating.
3. A carbon paper having an impression-yielding coating consisting of a compound of printer's copying ink, glycerin, spirits of turpentine, and spirits of camphor, and a coating 60 of finely powdered castile soap overlying said first mentioned coating.

In testimony whereof I affix my signature in presence of two witnesses.

WILLIAM L. WEST.

Witnesses:

ROBERT N. SPEER,  
E. R. INMAN.